

# UNITED STATES PATENT OFFICE.

JOHANN CHRISTIAN DUNTZE, OF FRANKFORT-ON-THE-MAIN, GERMANY.

## PROCESS OF PRODUCING COLORS ON GLASS SURFACES.

SPECIFICATION forming part of Letters Patent No. 508,873, dated November 14, 1893.

Application filed September 29, 1892. Serial No. 447,255. (No specimens.)

*To all whom it may concern:*

Be it known that I, JOHANN CHRISTIAN DUNTZE, residing at Frankfort-on-the-Main, in the Kingdom of Prussia and German Empire, have invented a new and useful Process of Producing Colors on Glass Surfaces, of which the following is a specification.

Notwithstanding numerous efforts no effective process has hitherto been discovered enabling manufacturers to reproduce on glass, any design in transparent colors, by mechanical means, for although it was found possible to apply colors to glass, yet these colors did not attain a sufficient transparency to form a perfect substitute for stained glass.

The subject of the present invention is a process of reprinting, or transfer, which will permit the accomplishment of the aforesaid end in an exceedingly simple and easy manner.

The design to be reproduced is outlined on the lithographic stone, zinc-plate or the like, in ordinary reprinting ink which is then transferred on to the well known transparent transfer-paper, viz., the so called "albuminous paper."

It is necessary in order to carry my invention into effect to reproduce each of the transparent colors separately upon transfer paper and transfer it upon the glass. The surface of the glass, which may be either flat or round is first carefully cleaned to remove dust and grease and the transfer sheet bearing the palest of the several colors to be employed in making up the picture, is laid upon the glass. The paper is laid face down upon the glass while yet unmoistened and is pressed against the surface of the glass with a soft brush or similar tool until it commences to adhere to the glass. The paper is then moistened on the back and again rubbed over with the soft

brush or tool. This process should terminate before the paper has given off all of its moisture and the paper while yet moist is pulled off of the glass leaving the transparent color upon the glass on the portions of the design where the color is desired. The color is then allowed to dry and will be found to be perfectly transparent. The transfer sheet bearing the next deeper color is then applied very carefully on exactly the same spot occupied by the other sheet so that lines of the design which they may have in common will exactly register and this color is applied in the same way, and allowed to dry. All of the colors necessary are thus applied successively and the colors are then covered with transparent varnish to preserve them, and add to their durability. The picture or pictures so produced will have the appearance of glass painting, as the transparent colors will be laid on one over the other producing tints and shades which could not be produced by the application of a single color. This forms a very serviceable imitation of stain glass and may be used for a variety of purposes, the process being comparatively simple and inexpensive.

What I claim, and desire to secure by Letters Patent, is—

The process of ornamenting glass which consists in printing in transparent colors upon separate transfer sheets, portions of the design, each color being printed upon a separate sheet and transferring said colors successively over one another onto the surface of the glass, substantially as described.

In witness whereof I have hereunto set my hand in presence of two witnesses.

JOHANN CHRISTIAN DUNTZE.

Witnesses:

ALVESTO S. HOGUE,  
JEAN GRUND.